

**1**

3,835,022

**ARCTIC DIESEL FUEL**

James A. Frayer, Pittsburgh, and Harry C. Stauffer, Cheswick, Pa., assignors to Gulf Research & Development Company, Pittsburgh, Pa.  
No Drawing. Filed Jan. 16, 1973, Ser. No. 324,147  
Int. Cl. C10I 1/08

U.S. Cl. 208—15

3 Claims

**ABSTRACT OF THE DISCLOSURE**

Kerosene and naphthenic petroleum oil fractions are blended to provide an arctic diesel fuel having a cloud point of at least as low as  $-45^{\circ}$  F., a pour point of at least as low as  $-50^{\circ}$  F., a cetane index of at least 40 and a distillation end point of at least  $625^{\circ}$  F.

**BACKGROUND OF THE INVENTION**

Standard refinery processes for the conversion of paraffinic or paraffinic-asphaltic crude oils into more valuable hydrocarbon fractions normally comprise fractionating or distilling the crude to recover separate streams of light gases, gasoline, kerosene, diesel oil, gas oil, and residual topped crude. The diesel oil fractions obtained from such processes normally have pour points above  $-10^{\circ}$  F. and distillation end points in the range of  $600^{\circ}$  to  $650^{\circ}$  F. Although acceptable as fuels for diesel engines in many geographical areas, it is evident that such fuels would not be acceptable in arctic regions or other geographical locations where diesel engines are operated in temperatures which are below the pour point of the diesel fuel.

To lower the pour point of these diesel oils, it is customary to blend kerosene with the diesel oil fraction. Paraffinic kerosene fractions will have substantially lower pour points than the higher distillation range diesel oil fraction with the precise pour point dependent upon the distillation range of the kerosene. For example, a kerosene fraction having an end point of  $500^{\circ}$  F. can be expected to have a pour point of about  $-50^{\circ}$  F. In the preparation of an arctic diesel fuel having a pour point of at least as low as  $-50^{\circ}$  F., it is evident that a blend of the kerosene and a diesel oil fraction described above to obtain the desired pour point would necessarily require that the blended product contain nearly 100 percent kerosene.

In addition to low cloud and pour points, arctic diesel fuels desirably are such that the distillation end point (as determined by ASTM D86) should be at least  $625^{\circ}$  F., and preferably in the range of  $625^{\circ}$  to  $650^{\circ}$  F. If a diesel fuel composition was prepared by blending a kerosene fraction with a diesel oil fraction as described in the above paragraph, the distillation end point of the blend would be substantially below  $625^{\circ}$  F.

Accordingly, an object of the invention is to provide an improved diesel fuel composition having a pour point substantially below the pour point of conventional paraffinic diesel oil fractions.

Another object of the invention is to provide a diesel fuel having a cloud point at least as low as  $-45^{\circ}$  F., a pour point of at least as low as  $-50^{\circ}$  F. and a distillation end point of at least  $625^{\circ}$  F.

Other objects, advantages and features of the invention will be readily apparent to those skilled in the art from the following description and appended claims.

**2****INVENTION**

A diesel fuel composition having a cloud point at least as low as  $-45^{\circ}$  F., a pour point of at least as low as  $-50^{\circ}$  F. and a distillation end point of at least  $625^{\circ}$  F. is obtained by preparing a blend comprising from 5 to 15 volume percent of a naphthenic petroleum oil and a kerosene.

**DESCRIPTION OF THE INVENTION**

In the preparation of diesel fuels for consumption in diesel engines there are specifications, in addition to cloud, pour, and distillation end point characteristic discussed above, which are employed to define a suitable arctic diesel fuel. For purposes of this invention, the term "arctic diesel fuel" as employed herein refers to a diesel fuel which has the following specifications:

|                                         |     |
|-----------------------------------------|-----|
| Pour point (ASTM 97), ° F., Maximum     | —50 |
| Cloud point (ASTM D2500), ° F., Maximum | —45 |
| Cetane index (D613), Minimum            | 40  |
| Distillation end point, ° F., Minimum   | 625 |

In preparing the novel diesel fuel compositions of this invention, a petroleum naphthenic oil fraction, as hereinafter described, is blended with a substantially paraffinic kerosene fraction. The kerosene which can be obtained from crude oil fraction by conventional distillation process will have a distillation range as determined by ASTM D86 from about  $310^{\circ}$  F. to about  $535^{\circ}$  F. and a flash point (as determined by ASTM D93) of at least  $120^{\circ}$  F. The cloud and pour point of the described paraffinic kerosene fraction will range from  $-40^{\circ}$  F. to  $-50^{\circ}$  F. and  $-45^{\circ}$  F. to  $-60^{\circ}$  F., respectively.

The naphthenic petroleum oil employed in preparing the novel blended compositions of this invention can be obtained from crude oil by conventional distillation process known in the art. The naphthenic compound should be comprised of at least 95 percent naphthenes in the saturate fraction and have a distillation range from about  $525^{\circ}$  to about  $800^{\circ}$  F. The cloud and pour points of the naphthenic component will generally be lower than  $-65^{\circ}$  F.

A suitable method for obtaining the highly naphthenic blend component of this invention can comprise fractionating a naphthenic crude oil to obtain a fraction having the above-described distillation range which shall have a paraffinic content of less than 5 volume percent. The naphthenic component can then be passed over hydrogenation catalyst in a conventional process where it is treated to improve its thermal stability and effect removal of sulfur compounds, nitrogen and other impurities if desired.

The kerosene and naphthenic petroleum oil components are blended together so as to form a diesel fuel composition containing from 5 to 15 percent by volume of the naphthenic component. The product blend will normally have a cloud point  $-55^{\circ}$  F. or below and a pour point of  $-60^{\circ}$  F. or below. The distillation end point of the distillate will normally range from  $625$  to  $650^{\circ}$  F. with the cetane index being at least 45.0.

The following example is presented to illustrate the objects and advantages of the invention. It is not intended, however, to limit the invention to the specific embodiments presented therein.

**3**  
**EXAMPLE**

An arctic diesel fuel composition was prepared by blending kerosene and 10 percent by volume of a petroleum naphthenic oil. The kerosene employed in the blend had the following properties:

|                    |      |
|--------------------|------|
| Gravity, °API      | 43.1 |
| Cloud Point, °F.   | —47  |
| Pour Point, °F.    | —55  |
| Cetane Index       | 46.3 |
| Distillation, °F.: |      |
| Overhead Point     | 333  |
| End Point          | 493  |
| 10%                | 363  |
| 30%                | 379  |
| 50%                | 401  |
| 70%                | 431  |
| 90%                | 465  |

The petroleum naphthenic oil employed in blend contained 100 percent naphthenes in the saturate fraction and had the following properties:

|                    |      |
|--------------------|------|
| Gravity, °API      | 25.6 |
| Cloud Point, °F.   | <—65 |
| Pour Point, °F.    | <—65 |
| Cetane Index       | 47.2 |
| Distillation, °F.: |      |
| Overhead Point     | —    |
| End Point          | 768  |
| 10%                | 564  |
| 30%                | 601  |
| 50%                | 639  |
| 70%                | 658  |
| 90%                | 691  |

The diesel fuel product blend had the following properties:

|                  |      |
|------------------|------|
| Gravity, °API    | 41.4 |
| Cloud Point, °F. | —60  |
| Pour Point, °F.  | —65  |
| Cetane Index     | 46.0 |

**4****Distillation, °F.:**

|                |     |
|----------------|-----|
| Overhead Point | 332 |
| End Point      | 633 |
| 10%            | 360 |
| 30%            | 382 |
| 50%            | 417 |
| 70%            | 453 |
| 90%            | 513 |

10 Although the invention has been described with reference to specific embodiments, references, and details, various modifications and changes will be apparent to one skilled in the art and are contemplated to be embraced in the invention.

15 We claim:

1. An arctic diesel fuel composition comprising a blend of a substantially paraffinic kerosene with from 5 to 15 volume percent of a naphthenic petroleum oil comprised of at least 95% naphthenes in the saturate fraction and having a distillation range from about 525 to about 800° F.

2. The composition of Claim 1 wherein the concentration of the naphthenic petroleum oil is about 10 percent by volume.

25 3. The composition of Claim 1 wherein the distillation range of the kerosene is in the range from about 330° F. to about 500° F.

**References Cited****UNITED STATES PATENTS**

|           |         |         |        |
|-----------|---------|---------|--------|
| 3,522,169 | 7/1970  | Ireland | 208—15 |
| 3,620,961 | 11/1971 | Ireland | 208—15 |

**OTHER REFERENCES**

Nelson: "Petroleum Refinery Engineering" 4th edition, 1958, pp. 56 to 58, 156 and 158 to 161, pub. McGraw-Hill Inc., N.Y., N.Y.

HERBERT LEVINE, Primary Examiner